

# United States Patent

Page et al.

[15] 3,655,533

[45] Apr. 11, 1972

[54] **ZINC ELECTROPLATING PROCESS  
AND ACIDIC ZINC FLUOBORATE  
ELECTROLYTE THEREFOR**

[72] Inventors: **Walter Page**, Convent, N.J.; **William R. Schevey**, Hawley, Pa.; **John E. Vander Mey**, Stirling, N.J.

[73] Assignee: **Allied Chemical Corporation**, New York, N.Y.

[22] Filed: **Nov. 12, 1970**

[21] Appl. No.: **89,068**

[52] U.S. Cl. .... **204/55 R**

[51] Int. Cl. .... **C23b 5/12**

[58] Field of Search .... **204/55 R**

[56] **References Cited**

UNITED STATES PATENTS

2,523,160 9/1950 Struyk et al.....204/45

2,537,032 1/1951 Chester et al. .... **204/55 R**  
2,807,585 9/1957 Gardner et al. .... **252/148**

FOREIGN PATENTS OR APPLICATIONS

1,109,479 6/1961 Germany..... **204/55 R**  
254,292 3/1970 U.S.S.R..... **20/55 R**

Primary Examiner—F. C. Edmundson  
Attorney—Jay P. Friedenson

[57] **ABSTRACT**

An acidic zinc electroplating bath comprising zinc fluoborate dissolved in an aqueous liquid containing as an iron- and metal oxide-deposition inhibitor a small effective amount of a mixture of a 4-hydroxy-, 4-alkyl- or aryl-, 5-acyl- or aroyl-piperidine and thiourea or N-substituted derivative thereof. The invention also includes an improved process for zinc-electroplating ferrous metals from such bath.

21 Claims, No Drawings

## ZINC ELECTROPLATING PROCESS AND ACIDIC ZINC FLUOBORATE ELECTROLYTE THEREFOR

## BACKGROUND OF THE INVENTION

This invention relates to a process for electrodepositing zinc from acidic zinc fluoborate plating baths and, more particularly, to a procedure for plating zinc on ferrous objects which inhibits co-plating of iron and deposition of iron and zinc oxides. The invention also includes a novel acidic zinc fluoborate bath for use in this process.

It is known to plate zinc onto ferrous metal objects, such as steel or iron rods, wires, strips and the like, from acid zinc fluoborate plating baths by directing an electric current through such electrolyte baths using zinc metal as the anode and the steel object to be plated as the cathode. One typical acidic zinc fluoborate plating electrolyte has been comprised of zinc fluoborate in aqueous solution, usually also containing ammonium chloride, and adjusted to an acidic pH, such as 3.0 to 3.5, with ammonium hydroxide. There are several serious disadvantages associated with use of such acidic zinc fluoborate baths in electroplating ferrous metal objects which limit the utilization of such baths in commercial zinc plating operations. For example, zinc electroplatings of ferrous metal from acidic zinc fluoborate baths are generally rough and coarse-grained in texture, rather than smooth and fine-grained as is desirable. Furthermore, the strongly corrosive fluoboric acid of the bath dissolves the ferrous metal cathode resulting in build-up of cationic iron in the electrolyte. The dissolved iron then co-plates with the zinc on the cathode resulting in an undesirable mixed plating of zinc and iron. Zinc plated ferrous metal articles, for example, steel strip, are generally fabricated into useful articles by cutting, stamping, drawing and forming operations. In order to withstand such operations without damage to the adhesion of the coating to the steel surface, it is essential that the electroplated zinc coating be ductile, tightly adhering and that it have a relatively low content of impurities, particularly iron co-deposited with zinc.

An additional disadvantage of conventional acidic zinc fluoroborate electroplating baths and processes also arises from aforementioned build-up of cationic iron in the electroplating electrolyte. It is found that conventional acidic zinc fluoroborate electroplating baths have a low tolerance for dissolved cationic iron. At electrolyte concentrations of cationic iron exceeding a certain low limit, say about 4 g. iron per liter of bath, the dissolved iron interferes with the normal plating of zinc resulting in a black spongy deposit of zinc and zinc oxide containing a small amount of iron oxides on the surface of the cathode, instead of the attractive white zinc coating normally obtained. As will be apparent to those skilled in the art, addition to the plating bath of a conventional iron anticorrosion agent, that is, an agent which inhibits corrosion of iron or steel by acids, is not an adequate remedy to the foregoing problems associated with dissolved cationic iron build-up, since such agents merely retard, rather than prevent, dissolution of iron by acidic substances.

It is, therefore, an object of the present invention to provide a process for electroplating zinc on ferrous metals from an acidic zinc fluoroborate electrolyte which minimizes the co-deposition of iron with the zinc on the ferrous metal cathode.

It is a further object of the invention to provide an acidic zinc fluoborate electroplating bath which tolerates larger than normal concentrations of cationic iron in the bath before unacceptable deposition of metal oxides occurs.

and/or a deposit of metal oxides occurs.

It is a still further object of the invention to provide an improved process and electrolyte for electroplating zinc on ferrous objects in a desirable fine grain of attractive appearance.

These and other objects and advantages will be apparent from the following description of our invention.

## SUMMARY OF THE INVENTION

The aforementioned disadvantages of prior art acidic zinc fluoborate electroplating baths and processes are overcome and the above objects are attained according to our invention.

wherein an acid zinc fluoborate electroplating bath is provided comprising zinc fluoborate dissolved in an acidic aqueous liquid containing a mixture of a 4-hydroxy-, 4-alkyl- or aryl-, 5-acyl- or aroyl-piperidine and thiourea or N-alkyl-, aryl- or aralkyl- substituted derivatives thereof in a small amount capable of promoting formation of an attractive fine-grained zinc coating, of inhibiting iron plating and of raising the tolerance of the bath toward dissolved iron so as to forestall cathode deposition of zinc and iron oxides.

It was highly surprising to discover, according to the invention, that the presence of mixtures of the aforementioned substituted piperidines and thioureas effectively inhibited the co-plating of iron with zinc on electroplating ferrous metals from acidic aqueous zinc fluoborate baths, as is illustrated below in Example 4. Such piperidine-thiourea mixtures have been disclosed by U.S. Pat. No. 2,807,585 as anti-corrosion agents for ferrous metals, that is, as inhibitors to retard dissolution of such metals by aqueous acids, which dissolution is an oxidation reaction. It was, therefore, surprising to discover that such mixtures in an electroplating environment inhibited the reverse reaction, namely, the electrochemical reduction of cationic iron to the free ferrous metal.

25 It was also surprising to discover, in accordance with the invention, that the present additive increases the tolerance of acidic aqueous zinc fluoborate electroplating baths toward dissolved cationic iron by as much as about 300 percent, as is illustrated below in Example 3. Unexpectedly also, the zinc 30 electroplatings on iron or steel obtained from an aqueous acidic zinc fluoborate electrolyte containing the present additive are of substantially finer grain and more attractive appearance than the corresponding zinc platings obtained from conventional aqueous acidic zinc fluoborate electrolytes devoid of this additive.

## DETAILED DESCRIPTION OF THE INVENTION AND THE PREFERRED EMBODIMENTS THEREOF

40 The substituted piperidine additives of the invention have the structural formula



wherein R is lower alkyl, lower cycloalkyl, aralkyl in which the alkylene moiety is methylene or vinylene and in which the aryl moiety is of the benzene or naphthalene series, hydrogen or a radical of the formula



60 and  $R_1$  is lower alkyl, aryl of the benzene or naphthalene series or aralkyl in which the alkylene moiety is methylene or vinylene and in which the aryl moiety is of the benzene or naphthalene series.

65 The designations "lower alkyl" and "lower cycloalkyl," employed in the above definition and hereinafter, refer to saturated radicals containing up to eight carbon atoms. The designation of aryl radicals or aryl moieties as being of the benzene or naphthalene series, as employed in the above definition and hereinafter, refers to phenyl or naphthyl radicals which may be unsubstituted or which contain, in addition to hydrogen, other conventional inert substituents such as lower alkyl, halogen, such as fluorine, chlorine and bromine, and lower alkoxy. By inert, we mean substituents which are inert to the acidic plating bath under electroplating conditions.

Typically, R of the above general structural formula (I) can be methyl, n-propyl, isopropyl, n-butyl, t-butyl, n-hexyl, n-octyl, benzyl, p-chlorobenzyl, 1-naphthylmethyl, cyclohexyl or cyclopentyl. Typically, R<sub>1</sub> can be methyl, ethyl, n-propyl, isopropyl, t-butyl, n-hexyl, n-octyl, phenyl, 1- or 2-naphthyl, benzyl, 1- or 2-naphthylmethyl, o-, m- or p-anisyl, o-, m- or p-chlorophenyl, o-, m- or p-chlorobenzyl or o-, m- or p-tolyl.

The substituted piperidines charged in accordance with the invention are known compounds disclosed in U.S. Pat. No. 2,807,585 and J. T. Pati et al., J. Org. Chem. 14 873 (1949), the pertinent subject matter of which patent and article are incorporated herein by reference.

Preferably, we employ a substituted piperidine of the above general formula in which R is a



radical. Still preferably, we employ a substituted piperidine in which R<sub>1</sub> is lower alkyl. An especially good result is obtained employing as the piperidine additive 1-acetylethyl-4-hydroxy-4-methyl-5-acetyl piperidine of the structure



The N,N-substituted thiourea charged in accordance with the invention has the following structural formula



wherein R<sub>2</sub> and R<sub>3</sub> are individually selected from lower alkyl radicals, lower cycloalkyl radicals, aryl radicals of the benzene or naphthalene series and aralkyl radicals wherein the alkylene moiety is methylene and the aryl moiety is of the benzene or naphthalene series.

Typical suitable thiourea additives include the following representative examples:

thiourea  
N-methyl thiourea  
N-phenyl thiourea  
N-p-tolyl thiourea  
N-benzyl thiourea  
N-(1-naphthyl)thiourea  
N-(2-naphthyl)thiourea  
N-(2-naphthylmethyl)thiourea  
N-(n-octyl) thiourea  
N,N'-di(n-octyl)thiourea  
N-(n-isopropyl)thiourea  
N-cyclohexylthiourea  
N,N'-dicyclohexylthiourea  
N,N'-dicyclooctylthiourea  
N-cyclopentylthiourea  
N,N'-dicyclopentylthiourea  
N,N'--(p-anisyl)thiourea  
N,N'--(p-tolyl)thiourea  
N-(phenyl)N'-(p-tolyl)thiourea  
N-(methyl)N'-(benzyl)thiourea  
N,N'-di(p-chlorobenzyl)thiourea  
N,N'-di(p-isopropylphenyl)thiourea  
N,N'-di(p-t-butylphenyl)thiourea  
N,N'-di(1-naphthyl)thiourea  
N-phenyl-N'(1-naphthyl)thiourea

- N-methyl-N'-ethyl thiourea  
N,N'-di(1-methylnaphthyl)thiourea  
N,N'-di(1-naphthylmethyl) thiourea  
N,N'-di(p-fluorophenyl)thiourea  
N,N'-di(m-tolyl)thiourea  
N,N'-di(o-tolyl)thiourea  
N,N'-di(p-[n-octyl]phenyl)thiourea  
N,N'-di(1-naphthyl)thiourea  
N,N'-di(p-xylyl)thiourea  
N,N'-di(m-xylyl)thiourea  
N,N'-di(o-xylyl)thiourea  
N,N'-di(2,4-dichlorobenzyl)thiourea  
N,N'-di(t-butyl)thiourea  
N,N'-di(p-bromobenzyl)thiourea  
N,N'-di(o-chlorophenyl)thiourea  
N,N'-di(p-fluorophenyl)thiourea  
Mixtures of these and equivalent thiourea compounds corresponding to the above general structural formula (III) may also be employed in the additive formulation of the invention.
- Preferably, we employ a thiourea wherein R<sub>2</sub> and R<sub>3</sub> are both aryl radicals of the benzene series. Use of N,N'-di(p-tolyl)thiourea as the thiourea additive provides an especially good result.
- The concentration of the mixture of substituted piperidine and thiourea compound which is required in the zinc fluoborate plating bath of the invention to inhibit iron plating, to produce a fine-grain zinc coating and to increase the tolerance of the electrolyte toward dissolved iron can be as small as about 0.004 g. per liter of the bath or less and preferably is about 0.03 to 0.2 g. per liter of bath. A concentration of 10 g. per liter or more of the substituted piperidine-thiourea mixture, however, can be employed in accordance with the invention.
- The proportion of the substituted piperidine compound and thiourea compound in the mixture charged to acidic zinc fluoborate electroplating baths, in accordance with the invention, can vary over a wide range. Thus, there can be employed as additive, mixtures containing from about 20 weight percent to about 80 weight percent of the substituted piperidine, the balance of the mixture being the thiourea compound. Preferably, the additive contains about 50 to 75 weight percent of the substituted piperidine compound.
- The aqueous zinc fluoborate electrolyte to which the inhibitor mixture is charged, in accordance with the invention, is conventional in the electroplating art. A preferred typical aqueous acid zinc fluoborate electrolyte to which the inhibitor mixture is charged in accordance with the invention has the following composition:
- | Ingredient Dissolved in the Bath | Concentration in Grams per Liter of Aqueous Bath                                           |
|----------------------------------|--------------------------------------------------------------------------------------------|
| zinc fluoborate                  | about 250 to 350, especially about 300                                                     |
| ammonium chloride                | about 20 to 40, especially about 40                                                        |
| ammonium fluoborate              | about 10 to 30, especially about 12                                                        |
| ammonium hydroxide               | an amount sufficient to provide a pH of about 3.0 to 3.5 at commencement of electroplating |
- Other suitable conventional aqueous acidic zinc fluoborate electrolyte formulations for electroplating zinc on ferrous metals in the presence of the above-described inhibitor mixture will be apparent to those skilled in the art.
- The electrogalvanizing process of the invention can be carried out employing a zinc fluoborate bath of the above-described type wherein the inhibitor mixture is dispersed or advantageously dissolved. A zinc anode is inserted in the bath and the ferrous metal object to be plated is made the cathode. In accordance with conventional electroplating procedures, the temperature of the bath during plating can conveniently range from about ambient temperature to about 200° F., but advantageously is about 170° to 190° F., especially about 180° F. Desirably also, the bath is well-agitated during the electroplating operation. Zinc electroplating, in accordance with the invention, can be carried out batchwise or in a continuous fashion.

To minimize corrosion of the zinc anode by the acidic bath, the electroplating operation is preferably carried out at a relatively high current density of between about 700 amperes per square foot of anode (ASF, anode) and about 3,000 amperes per square foot of anode, still preferably at an anode current density of about 1,000 to 2,000 ASF. As is apparent from a comparison of the results of experiments (a) and (b) of Example 1 below, electroplating from acidic zinc fluoborate baths at relatively low anode current densities, say about 5 to 700 ASF, causes rapid corrosion of the zinc anode which becomes blackened by a deposit of zinc oxide. As the pH of the bath rises to above about 4 during the plating process, as is normal in electroplating from such baths, the large quantity of dissolved zinc ion built up in the bath as a result of the aforesaid anode corrosion precipitates as a zinc hydroxy-fluoborate sludge. This sludge migrates to the ferrous metal cathode forming a loosely adherent layer on the cathode which terminates the plating operation. As is apparent from the results of Example 1(b) below, plating from zinc fluoborate baths at anode current densities above about 700 ASF eliminates the aforementioned blackening of the anode and minimizes, but does not completely eliminate, precipitation of zinc hydroxy-fluoborate. To eliminate the latter undesirable effect, in accordance with a particularly preferred mode of operation, about 1 to 5 percent, advantageously about 2 to 5 percent, of the aforementioned high density current, which is normally delivered to the zinc anode, is shunted, variably if desired, through an inert carbon anode inserted in the bath while maintaining the overall bath efficiency during the plating operation at about 100 percent, that is at  $100 \pm 3$  percent, advantageously at  $100 \pm 1$  percent. Current shunting, which can

respectively, in the zinc electroplating of steel from a conventional aqueous acidic zinc fluoborate bath.

## EXAMPLE 1

Two zinc-plating baths, (a) and (b), are prepared having the following composition:

| 10                             | Ingredient | Grams/Liter of Aqueous Solution |
|--------------------------------|------------|---------------------------------|
| zinc fluoborate $[Zn(BF_4)_2]$ | 300*       |                                 |
| ammonium chloride              | 30         |                                 |
| ammonium fluoborate            | 12         |                                 |

\*Equivalent to 81 grams of zinc per liter.

The pH of each bath is adjusted to 3 to 3.5 by addition of ammonium hydroxide. An anode of zinc metal and a cathode 20 of strip steel are inserted into each bath. In order to determine the efficiencies of the anode and cathode in the above baths when operating at various current densities, a current of 2,800 coulombs is passed through each bath, the current through bath (a) having a density of 250 amperes per square foot of anode, the current through bath (b) having a density of 750 amperes per square foot of anode. Amounts of zinc released from the anodes and electrodeposited on the cathodes are measured and compared with the theoretical values calculated for these conditions. The temperature of the plating baths during the electroplating operation is 180°.

Results, which represent an average of three replications at each current density, are shown in Table I below:

TABLE I.—Efficiencies of zinc fluoborate plating baths at 250 ASF and 750 ASF current density.

| Bath     | Theoretical wt. of zinc to be transferred | Anode actual wt. loss, grams | Efficiency of anode, percent | Cathode actual wt. gain, grams | Efficiency of cathode, percent | Bath efficiency ratio  |
|----------|-------------------------------------------|------------------------------|------------------------------|--------------------------------|--------------------------------|------------------------|
| (a)----- | 250                                       | 0.9482                       | 1.0112                       | 107.7                          | 0.9128                         | 96.3 <sup>1</sup> 90.3 |
| (b)----- | 750                                       | 0.9482                       | 0.9551                       | 100.7                          | 0.9168                         | 96.7 <sup>2</sup> 96.0 |

<sup>1</sup> The zinc anode rapidly corroded and developed a black zinc oxide coating as the bath pH rose to 4. On continued operation at these conditions, a heavy sludge of zinc hydroxy-forming a loosely adherent layer thereon, terminating the plating process.

<sup>2</sup> The zinc anode remains clear of oxide deposits as the bath pH rises to 4, indicating a diminished degree of anode corrosion. On continued operation at these conditions above pH 4, some zinc hydroxyfluoborate precipitates.

be carried out in a continuous or semi-continuous manner during plating, maintains the concentration of zinc ion dissolved in the bath within about 10 weight percent of the initial zinc concentration of the electrolyte, thereby preventing any substantial accumulation of zinc ion in the bath and resultant undesirable precipitation of zinc hydroxy-fluoborate. Since only about 95-99 percent of the current normally charged to the zinc anode passes through the zinc anode during current shunting, the corrosion of the latter anode is minimized also.

The present electrogalvanizing process employing the aforementioned preferred process modifications of high density current and current shunting is especially suitable for high-speed continuous zinc plating of steel strip, sheet, wire and the like to obtain platings of improved texture, appearance and diminished co-plated iron content.

In the following examples, which serve to illustrate our invention, temperatures are in degrees Fahrenheit.

The following Examples 1 and 2 illustrate the effects of low and high current density and the effect of current shunting,

60 It is apparent from the data of Table I that use of an anode current of relatively high density, that is, a current having a density above about 700 ASF, while providing a bath efficiency substantially equivalent to that obtained employing a current of relatively low density, minimizes anode corrosion. However, use of the high density current nevertheless results in some build-up of cationic zinc in the bath, as is indicated by the precipitation of some zinc hydroxyfluoborate in bath (b), at a bath pH above about 4.

## EXAMPLE 2

70 In two experiments, (a) and (b), the procedure of Example 1 is repeated substantially as described, employing a current having a density of 750 ASF, except that in each experiment different portions of the anode current are shunted through an inert carbon anode inserted in the bath. In the first experiment (a), 2 percent of the anode current is shunted through the carbon anode; in the second experiment (b), 5 percent of the anode current is shunted through the inert carbon anode.

Resulting efficiencies of these experiments are tabulated in Table II below:

TABLE II.--EFFICIENCIES OF ZINC ANODE, CATHODE AND BATH WHEN SHUNTING 2% AND 5% OF CURRENT THROUGH CARBON ANODES WHEN OPERATING AT 750 ASF.

| Experiment | Percent current shunted to carbon anode | Theoretical wt. of zinc to be transferred | Zinc actual wt. loss, grams | Efficiency of anode, percent | Cathode, wt. gain, grams | Efficiency of cathode, percent | Bath efficiency, percent |
|------------|-----------------------------------------|-------------------------------------------|-----------------------------|------------------------------|--------------------------|--------------------------------|--------------------------|
| (a)-----   | 2                                       | 0.9482                                    | 0.9379                      | 98.9                         | 0.9477                   | 99.9                           | 101.0                    |
| (b)-----   | 5                                       | 0.9482                                    | 0.8951                      | 94.4                         | 0.9461                   | 99.7                           | 105.5                    |

<sup>1</sup> No zinc hydroxyfluoborate precipitates.

It is apparent from Table II that the bath efficiencies are substantially increased by shunting up to 5 percent of the current normally passed through the zinc anode through an inert carbon anode inserted in the bath. As is further indicated by Table II, the anode and cathode efficiencies of experiment (a) are substantially balanced when about 2 percent of the current at 750 asf is shunted through the inert carbon anode with about 98 percent passing through the zinc anode, the overall bath efficiency being 101.0 percent, that is, about 100 percent. In experiment (b) wherein 5 percent of the current is shunted, the bath efficiency is considerably above 100 percent, that is, substantially more zinc is being plated out on the cathode than is being released into the bath from the zinc anode.

It is apparent from the foregoing experiments that by increasing or decreasing the proportion of current shunted through the inert carbon anodes, the operator can diminish or increase the zinc ion concentration in the bath and thereby maintain said concentration within about 10 percent of the concentration of zinc ion initially charged.

The following Examples 3-20 illustrate the novel acidic aqueous zinc fluoborate bath of the invention containing a mixture of a substituted piperidine and thiourea compound described above and the use of this novel bath in electroplating zinc on ferrous metals.

### EXAMPLE 3

A series of eight baths as described in example 1 are prepared, and to each is added 0.25 gram per liter of a commercial mixture containing about 70 weight percent of inert inorganic salt filler and about 30 weight percent of a mixture of about 66.7 weight percent of a substituted piperidine corresponding to the structural formula (I) above and about 33.3 weight percent of N,N'-di(p-tolyl)thiourea (Rhodine 115, American Chemical Paint Co.). This group of baths is designated Group X. Another group of five baths, designated Group Y, identical to those of Group X except that no piperidine-thiourea mixture is added, is prepared. Cationic iron in the form of ferrous fluoborate is charged to each of the baths in Group X in varying amounts from 1 to 15 grams of Fe<sup>++</sup> per liter, as indicated in Table III below. In a similar manner, ferrous fluoborate is charged to each of the baths in Group Y to provide bath concentrations of Fe<sup>++</sup> varying from 1 to 5 grams per liter, as indicated in Table IV below. After insertion of zinc anodes and steel cathode into each bath, both anodes and cathodes being of the same surface area, currents are passed through each bath at a current density of 1,000 amperes per square foot of anode, at a temperature of 180°, and at an initial bath pH OF 3.5. The results of plating from Group X baths and from Group Y baths are set forth in Table III and Table IV, respectively.

TABLE III  
Zinc Electroplatings from Acidic Aqueous  
Zinc Fluoborate Baths of Group X Containing  
0.075 Grams per Liter of Substituted  
Piperidine-N,N'-di(p-tolyl)Thiourea Additive

| Bath           | Grams Fe <sup>++</sup> per liter of Bath | Character of Plating on Steel Cathode                                                    |
|----------------|------------------------------------------|------------------------------------------------------------------------------------------|
| X <sub>a</sub> | 1                                        | white metallic finish indicative of satisfactory zinc plating                            |
| X <sub>b</sub> | 2                                        | as in X <sub>a</sub> , above                                                             |
| X <sub>c</sub> | 3                                        | as in X <sub>a</sub> , above                                                             |
| X <sub>d</sub> | 5                                        | as in X <sub>a</sub> , above                                                             |
| X <sub>e</sub> | 8                                        | as in X <sub>a</sub> , above                                                             |
| X <sub>f</sub> | 10                                       | as in X <sub>a</sub> , above                                                             |
| X <sub>g</sub> | 12                                       | as in X <sub>a</sub> , above                                                             |
| X <sub>h</sub> | 15                                       | black spongy coating indicative of deposition of zinc and iron oxides together with zinc |

TABLE IV

Zinc Electroplatings from Acidic Aqueous  
Zinc Fluoborate Baths of Group Y Devoid  
of Substituted Piperidine-N,N'-di(p-tolyl)-  
Thiourea Additive

| Bath           | Grams Fe <sup>++</sup> per liter of Bath | Character of Plating on Steel Cathode                                                        |
|----------------|------------------------------------------|----------------------------------------------------------------------------------------------|
| Y <sub>a</sub> | 1                                        | white metallic plating indicative of satisfactory zinc plating                               |
| Y <sub>b</sub> | 2                                        | as in Y <sub>a</sub> above                                                                   |
| Y <sub>c</sub> | 3                                        | as in Y <sub>a</sub> above                                                                   |
| Y <sub>d</sub> | 4                                        | as in Y <sub>a</sub> above                                                                   |
| Y <sub>e</sub> | 5                                        | black spongy coating indicative of the deposition of zinc and iron oxides together with zinc |

From a comparison of Tables III and IV, it is apparent that the presence of the substituted piperidine-N,N'-di(p-tolyl)thiourea mixture in the plating bath raises the tolerance of the bath toward dissolved cationic iron by at least about 300 percent. In other words, it is possible to obtain satisfactory zinc electroplatings on ferrous metal cathodes from acidic aqueous zinc fluoborate baths containing as much as 12 grams per liter Fe<sup>++</sup> in the presence of the additive, whereas elec-

troplating from such baths in the absence of the additive, at a concentration of more than about 4 grams per liter  $Fe^{++}$  in the bath results in a black deposit of metal oxides at the cathode, that is, prevents obtainment of a satisfactory zinc plating.

#### EXAMPLE 4

Three acidic aqueous zinc fluoborate plating baths (a), (b) and (c) of the composition described in Example 1 are prepared. To baths (a) and (b) is added 0.25 gram per liter (corresponding to 0.075 gram per liter of bath, of active ingredients) of the substituted piperidine— $N,N'$ -di(p-tolyl)thiourea mixture of Example 3. Ferrous fluoborate is charged to each bath to provide the concentrations of  $Fe^{++}$  indicated in Table V below. Zinc anodes and nickel cathode are inserted in each bath, nickel cathode being employed in place of ferrous metal cathodes in order to facilitate removal of resultant zinc platings for analysis. Currents of 1,000 amperes per square foot of anode are passed through each bath for 30 minutes. The resultant platings are then stripped from each cathode and analyzed for total iron content. The results of these experiments are presented in Table V below.

TABLE V

| Bath | Concentration of Substituted Piperidine— $N,N'$ -di(p-tolyl)Thiourea Additive in Bath (grams per liter) | Initial concentration of $Fe^{++}$ in Bath (grams per liter) | Tons in Plating (weight percent) |
|------|---------------------------------------------------------------------------------------------------------|--------------------------------------------------------------|----------------------------------|
| (a)  | 0.075                                                                                                   | 5.9                                                          | 0.120                            |
| (b)  | 0.075                                                                                                   | 12.0                                                         | 0.178                            |
| (c)  | 0                                                                                                       | 5.9                                                          | 0.202                            |

bath at about 180° at an anode current density of 1,000 asf while about 2 percent of the current is continuously shunted through the carbon anode, in accordance with the technique of Example 2, to maintain the zinc ion concentration in the bath at about  $81 \pm 5$  grams per liter. Passage of the current is continued for 10.5 seconds at a cathode current density of 1,000 asf to obtain a plating of  $\frac{1}{8}$  ounce of zinc per square foot on the cathode. The resultant zinc plating is smooth, fine-grained and attractive in appearance.

10

#### EXAMPLE 6

The procedure of Example 5 is repeated substantially as described, omitting the addition of the substituted-piperidine-substituted thiourea mixture to the bath. The resultant zinc plating is rough, coarse-grained and unattractive in appearance.

15

#### EXAMPLE 7

The procedure of Example 5 is repeated substantially as described, except that the electroplating bath contains 0.1 gram per liter of 1-acetylethyl-4-hydroxy-4-methyl-5-acetyl piperidine having the structural formula (II) above and 0.1 gram per liter of  $N,N'$ -di(p-tolyl)thiourea in place of the inhibitor mixture charged in Example 5. An excellent plating of zinc on steel substantially similar to the product of Example 5 is obtained.

20

In the following Examples 8-20, which are summarized in Table VI below, excellent electroplatings of zinc on ferrous metals are obtained utilizing the plating technique of Example 7 with various other substituted piperidine and thiourea additives, the structures of which are listed in each tabulated example.

TABLE VI

| Example: | Substituted piperidine of general structural Formula (I) above |                                             | Thiourea of general structural Formula (III) above |                        |
|----------|----------------------------------------------------------------|---------------------------------------------|----------------------------------------------------|------------------------|
|          | R =                                                            | R <sub>1</sub> =                            | R <sub>2</sub> =                                   | R <sub>3</sub> =       |
| 8.       | $-\text{CH}_2\text{CH}_2\text{C}=\text{R}_1$                   | $-\text{C}_2\text{H}_5$                     | Benzyl                                             | Benzyl                 |
| 9.       | $\text{O}$                                                     |                                             |                                                    |                        |
| 10.      | Cyclohexyl                                                     | $-\text{CH}_3$                              | $\text{CH}_3$                                      | $\text{C}_2\text{H}_5$ |
| 11.      | $-\text{CH}_3$                                                 | Phenyl                                      | n-Octyl                                            | H                      |
| 12.      | H                                                              | $\text{C}_6\text{H}_4-\text{CH}=\text{CH}-$ | Cyclohexyl                                         | Cyclohexyl             |
| 13.      | n-Butyl                                                        | Phenyl                                      | H                                                  | Isopropyl              |
| 14.      | Benzyl                                                         | Phenyl                                      | Isopropyl                                          | Isopropyl              |
|          | $-\text{CH}_2\text{CH}_2\text{C}=\text{R}_1$                   | $\text{O}$                                  | Phenyl                                             | Phenyl                 |
| 15.      | $\text{O}$                                                     |                                             |                                                    |                        |
| 16.      | $-\text{CH}_2\text{CH}_2\text{C}=\text{R}_1$                   | n-Octyl                                     | 1-naphthylmethyl                                   | 1-naphthylmethyl       |
| 17.      | $\text{O}$                                                     |                                             |                                                    |                        |
| 18.      | 1-naphthyl                                                     | 1-naphthyl                                  | p-Tolyl                                            | H                      |
| 19.      | n-Octyl                                                        | 2-naphthylmethyl                            | p-Chlorobenzyl                                     | p-Chlorobenzyl         |
| 20.      | Benzyl                                                         | Benzyl                                      | p-Xylyl                                            | p-Xylyl                |
|          | $-\text{CH}_2\text{CH}_2\text{C}=\text{R}_1$                   | $\text{O}$                                  | p-Anisyl                                           | p-Anisyl               |
|          | $\text{O}$                                                     |                                             | H                                                  | H                      |
|          |                                                                |                                             |                                                    |                        |

It is apparent from Table V that the presence of the substituted piperidine-substituted thiourea additive reduces the amount of iron co-plated with zinc by more than about 40 weight percent when the zinc fluoborate plating bath contains 5.9 grams per liter dissolved cationic iron.

#### EXAMPLE 5

A 30 liter zinc fluoborate plating bath of the composition described in Example 1 is prepared. To the bath is charged the substituted piperidine— $N,N'$ -di(p-tolyl)thiourea mixture of Example 3 in an amount equivalent to 0.25 gram per liter of bath (corresponding to 0.075 gram per liter active ingredients). A zinc anode, an inert carbon anode and a steel cathode are inserted in the bath. Current is passed through the

We claim:

1. A zinc electroplating bath comprising zinc fluoborate dissolved in an aqueous acidic liquid containing as an iron- and metal-oxide deposition inhibitor a small effective amount of a mixture of

a. a piperidine of the formula:



70

75

wherein R is lower alkyl, lower cycloalkyl, aralkyl in which the alkylene moiety is methylene or vinylene and in which the aryl moiety is of the benzene or naphthalene series, hydrogen, or a radical of the formula:

5



and R<sub>1</sub> is lower alkyl, aryl of the benzene or naphthalene series, or aralkyl in which the alkylene moiety is methylene or vinylene and in which the aryl moiety is of the benzene or naphthalene series, and

b. a thiourea of the formula:

15



wherein R<sub>2</sub> and R<sub>3</sub> are independently selected from hydrogen, lower alkyl, lower cycloalkyl, aryl of the benzene and naphthalene series and aralkyl in which the alkylene moiety is methylene and in which the aryl moiety is of the benzene or naphthalene series, the weight proportion of the piperidine in said mixture being about 20 to about 80 percent.

2. A zinc electroplating bath as claimed in claim 1 wherein the concentration of the inhibitor mixture is about 0.004 to 10 grams per liter of the bath.

3. A zinc electroplating bath as claimed in claim 2 wherein the concentration of the inhibitor mixture is about 0.03 to 0.2 gram per liter of the bath.

4. A zinc electroplating bath as claimed in claim 1 wherein the weight proportion of the piperidine in the inhibitor mixture is about 50 to 75 percent.

5. A zinc electroplating bath as claimed in claim 1 wherein R is



40

and R<sub>1</sub> is lower alkyl.

6. A zinc electroplating bath as claimed in claim 1 wherein R<sub>2</sub> and R<sub>3</sub> are both aryl radicals of the benzene series.

7. A zinc electroplating bath as claimed in claim 5 wherein the piperidine is 1-acetylethyl-4-hydroxy-4-methyl-5-acetyl-piperidine and the thiourea is N,N'-di(p-tolyl)thiourea.

8. A zinc electroplating bath as claimed in claim 1 which contains in solution about 250 to 350 grams per liter of bath of zinc fluoborate, about 20 to 40 grams per liter of bath of ammonium chloride, about 10 to 30 grams per liter of bath of ammonium fluoborate, an amount of ammonium hydroxide sufficient to provide a bath pH of about 3.0 to 3.5 and from about 0.03 to 0.2 gram per liter of bath of the mixture of the piperidine and the thiourea wherein the weight proportion of the piperidine is about 50 to 75 percent.

9. In the process of electroplating zinc on a ferrous metal cathode from an aqueous acidic zinc fluoborate bath employing a zinc anode, the improvement which consists in electroplating from a bath containing as an iron- and metal-oxide deposition inhibitor a small effective amount of a mixture of

a. a piperidine of the formula:



wherein R is lower alkyl, lower cycloalkyl, aralkyl in which the alkylene moiety is methylene or vinylene and in which

the aryl moiety is of the benzene or naphthalene series, hydrogen or a radical of the formula:



and R<sub>1</sub> is lower alkyl, aryl of the benzene or naphthalene series or aralkyl in which the alkylene moiety is methylene or vinylene and in which the aryl moiety is of the benzene or naphthalene series, and

b. a thiourea of the formula:



wherein R<sub>2</sub> and R<sub>3</sub> are independently selected from hydrogen, lower alkyl, lower cycloalkyl, aryl of the benzene or naphthalene series or aralkyl in which the alkylene radical is methylene and in which the aryl moiety is of the benzene or naphthalene series,

the weight proportion of the piperidine in said mixture being about 20 to about 80 percent.

10. An electroplating process as claimed in claim 9 wherein the concentration of the inhibitor mixture is about 0.004 to 10 grams per liter of the bath.

11. An electroplating process as claimed in claim 10 wherein the concentration of the inhibitor mixture is about 0.03 to 0.2 gram per liter of the bath.

12. An electroplating process as claimed in claim 9 wherein the weight proportion of the piperidine in the inhibitor mixture is about 50 to 75 weight percent.

13. An electroplating process as claimed in claim 9 wherein R is



and R<sub>1</sub> is lower alkyl.

14. An electroplating process as claimed in claim 9 wherein R<sub>2</sub> and R<sub>3</sub> are both aryl radicals of the benzene series.

15. An electroplating process as claimed in claim 13 wherein the piperidine is 1-acetylethyl-4-hydroxy-4-methyl-5-acetyl-piperidine and the thiourea is N,N'-di(p-tolyl)thiourea.

16. An electroplating process as claimed in claim 9 wherein the current density is between about 700 and about 3,000 amperes per square foot of anode.

17. An electroplating process as claimed in claim 16 wherein the current density is between about 1,000 and about 2,000 amperes per square foot of anode.

18. An electroplating process as claimed in claim 16 wherein about 1 to 5 percent of the current normally delivered to the zinc anode is shunted continuously or semi-continuously through an inert carbon anode inserted in the bath while maintaining the bath efficiency at about 100 percent.

19. An electroplating process as claimed in claim 18 wherein about 2 to 5 percent of the current is shunted through an inert carbon anode.

20. An electroplating process as claimed in claim 19 wherein the bath contains in solution about 250 to 350 grams per liter of bath of zinc fluoborate, about 20 to 40 grams per liter of bath of ammonium chloride, about 10 to 30 grams per liter of bath of ammonium fluoborate, an amount of ammonium hydroxide to provide an initial bath pH of about 3.0 to 3.5 and from about 0.03 to 0.2 grams per liter of bath of the mixture of the piperidine and the thiourea wherein the weight proportion of the piperidine is about 50 to about 75 percent, the electroplating being carried out at a temperature of about 170° to 190° F.

21. Ferrous metal plated with zinc in accordance with the process of claim 9.

\* \* \* \* \*